# EUROPEAN PATENT SPECIFICATION

(11) **EP 0 558 308 B1**
(45) Date of publication and mention of the grant of the patent: **10.05.1995**
(21) Application number: 93301385.6
(22) Date of filing: 24.02.1993
(51) Int. Cl.: H01J 1/34, H01J 40/06

(54) **Photoelectron emitting structure, and electron tube and photodetecting device using the photoelectron emitting structure**
Fotoelektronen emittierende Struktur und Elektronenröhre und Fotodetektorvorrichtung zur Verwendung der Fotoelektronen emittierenden Struktur
Structure émettrice de photoélectrons et tube à électrons et dispositif photodétecteur utilisant cette structure

(30) Priority: 25.02.1992 JP 37823/92
(43) Date of publication of application: 01.09.1993
(73) Proprietor: HAMAMATSU PHOTONICS K.K., Shizuoka-ken (JP)
(72) Inventor: Niigaki, Minoru, c/o Hamamatsu Photonics K. K., Hamamatsu-shi, Shizuoka-ken (JP)
(74) Representative: Burke, Steven David

(56) References cited:
- GB-A- 2 213 634
- US-A- 4 015 284
- US-A- 4 749 903
- APPLIED PHYSICS LETTERS. vol. 58, no. 14, 8 April 1991, NEW YORK US pages 1551- 1553 B F LEVINE ET AL. 'Photovoltaic GaAs quantum well infrared detectors at 4.3um using indirect AlxGa1-x barriers'

## Description

### BACKGROUND OF THE INVENTION

### Field of the Invention

This invention relates to a photoelectron emitting structure which emits photoelectrons by the incidence of photons, and an electron tube and a photodetecting device using the photoelectron emitting structure.

### Related Background Art

The art using semiconductor multi-layer films as a photoabsorbing layer for the end of providing a highly efficient photoelectron emitting structure are disclosed in Japanese Patent Laid-Open Publication No. 133634/1987 and 133633/1987. A first conventional photoelectron emitting structure disclosed in Japanese Patent Laid-Open Publication No. 133633/1987 has the energy band shown in FIG. 1. A narrow-energy gap film 6 has a sufficient thickness (below 300 Å) to absorb incident photons and generate photoelectrons. A wide-energy gap film 7 is thin (below 45 Å) enough to pass photoelectrons by the tunnel effect. The films 6, 7 are alternately laid one on the other in a photoelectron emitting structure. This photoelectron emitting structure uses the effect that the alternate superposition of two kinds of films increases a photoabsorbing coefficient for the incident photons in comparison with that of a conventional photoabsorbing layer consisted of homogeneous semiconductive materials. To efficiently lead photoelectrons generated by the incident photons to a photoemitting surface, a thickness of the wide-energy gap film 7 which is a barrier has to be thin enough, and practically has to be as thin as below 45 Å. Only those of the generated photoelectrons which have successfully passed the wider-energy gap film 7 owing to the tunnel effect arrive at the photoemitting surface to be emitted to a vacuum through a CsₓO_{y} film 8 formed on the photoemitting surface. In this photoelectron emitting structure, the photoemission efficiency is achieved by absorbing the incident photons and generating electron-hole pairs between the valence band and the conduction band of the narrower-energy gap film 6. A second conventional photoelectron emitting structure disclosed in Japanese Patent Laid-Open Publication No. 133634/1987 has the energy band structure of FIG. 2. In the energy band structure of this photoelectron emitting structure a narrower-energy gap film 9 has a smaller film thickness than the film 6 of the first conventional photoelectron emitting structure. In this photoelectron emitting structure as well, the absorption of the incident photons, and the generation of electron-hole pairs take place between the valence band and the conduction band of the narrower-energy gap film 9, emitting photoelectrons from a CsₓO_{y} film 11 for the improvement of photoemitting efficiency.

A long-wavelength photodetecting device using a quantum well structure is reported by B. F. Levine (Appl. Phys. Lett. 58(14) 1991). The band structure of the conduction band of this photodetecting device (a third conventional photoelectron emitting structure) is as shown in FIG. 3. Incident photons are absorbed between sub-bands of the conduction band formed in a narrow-energy gap film 12 which functions as the potential well, and photoelectrons are generated. In this case, the generated photoelectrons transfer through the X-valley of the conduction band of a wider-energy gap film 13 which functions as the potential barrier. In such photodetector, it is general that since the photoelectrons are detected as signals when they arrive at the electrode formed on the surface, electric fields formed inside the semiconductor device is small, and such photodetector is operated at biases as low as possible for suppressing noises as low as possible.

But the first conventional photoelectron emitting structure has an intrinsic problem. That is, as a thickness of the small-energy gap film 6 is decreased, sub-bands are formed due to the quantum effect both in the valence band and the conduction band, and a threshold for the incident photon absorption rises. As a result, incident long-wavelength photons cannot be absorbed.

In the second conventional photoelectron emitting structure, because of the thinness of the narrow-energy gap film 9, an energy difference E_{sg} between a sub-band of the valence band and a sub-band of the conduction band is larger than a band gap E_{g}, and as a result, an absorbed threshold wavelength of the incident photons is short.

In the third conventional photoemitting surface (the photodetecting device), as high dark currents is generated, the photoemitting surface has to be used at a remarkably low temperature by cooling down with liquid nitrogen or the like. As a result, it is difficult to be used in a general device as used at a room temperature.

### SUMMARY OF THE INVENTION

It would be desirable to solve the above-described problems. In the photoelectron emitting structure according to this invention, photoelectrons are emitted from a emitting surface by incident photons on a photoabsorbing layer, which is formed of a semiconductor multi-layer comprising a plurality of semiconductor films including a first semiconductor film and a second semiconductor film. The first semiconductor film with a narrow energy gap is formed in a thickness of below 300 Å which allows an electron state to be quantized. The second semiconductor film with a wide energy gap is formed in a thickness of above 45 Å which does not allow electrons to pass the second semiconductor film owing to the tunnel effect. The absorption of the incident photons and the generation of electron-hole pairs takes place between sub-bands of a conduction band or between a sub-band and a bottom of the conduction band of said first semiconductor film with the narrow energy gap, generated photoelectrons are accelerated by an internal electric field to transit to a higher energy band.

The photoelectrons which have been excited to a lowest energy level of the conduction band are energized to transit to a higher energy level, and are accelerated by the internal electric field.

An energy difference between lowest energy levels of the conduction bands formed in the respective semiconductor films making up the semiconductor multi-layer is smaller than a narrowest energy gap among energy gaps between bands of the respective semiconductor films themselves.

According to this invention, the absorption of the incident photons, and the generation of photoelectrons take place between the sub-bands of the conduction band of the first semiconductor film, or between the bottom of the conduction band and the sub-band. As a result, the photoelectron emitting structure has a sensitivity to the incident light of longer wavelengths than wavelengths corresponding to an energy gap of the used semiconductors. The generated photoelectrons are accelerated by an inside electric field to be easily emitted into a vacuum.

Accordingly, the photoelectron emitting structure according to this invention has much improved sensitivity in comparison with the conventional photoelectron emitting structures, and it is possible to set its threshold wavelength at a much longer wavelength.

Electron tubes using such photoelectron emitting structure are operative up to relatively high temperatures, and in comparison with the conventional photoelectron emitting structures, such photoelectron emitting structure exhibits very high sensitivity especially in a long-wavelength range.

Optional designs of the kinds and structure of the semiconductor multi-layer constituting the photoabsorbing layer of the photoelectron emitting structure according to this invention make the photoelectron emitting structure sensitive to a wide range from long to short wavelengths.

The present invention will become more fully understood from the detailed description given hereinbelow and the accompanying drawings which are given by way of illustration only, and thus are not to be considered as limiting the present invention.

Further scope of applicability of the present invention will become apparent from the detailed description given hereinafter. However, it should be understood that the detailed description and specific examples, while indicating preferred embodiments of the invention, are given by way of illustration only, since various changes and modifications within the spirit and scope of the invention will become apparent to those skilled in the art form this detailed description.

### BRIEF DESCRIPTION OF THE DRAWINGS

FIG. 1 is a view of the band structure of the first conventional photoelectron emitting structure.

FIG. 2 is a view of the band structure of the second conventional photoelectron emitting structure.

FIG. 3 is a view of the band structure of the third conventional photoelectron emitting structure.

FIG. 4 is a sectional structural view of the photoelectron emitting structure according to one embodiment of this invention.

FIG. 5 is a view of a band structure of the photoelectron emitting structure according to the embodiment of FIG. 4 with no bias applied to.

FIG. 6 is a view of a band structure of the photoelectron emitting structure according to the embodiment of FIG. 4 with a bias applied to.

FIG. 7 is a sectional view of a side-on photomultiplier using the photoelectron emitting structure according to this invention.

FIG. 8 is a sectional view of a head-on photomultiplier using the photoelectron emitting structure according to this invention.

FIG. 9 is a sectional view of an image intensifier using the photoelectron emitting,structure according to this invention.

### DESCRIPTION OF THE PREFERRED EMBODIMENT

The photoelectron emitting structure according to one embodiment of this invention will be explained with reference to FIG. 4.

A photoabsorbing layer 22 is formed on a P⁺-GaAs substrate 21. The photoabsorbing layer 22 comprises 40 undoped GaAs films of a 30 Å-thickness 22a and 40 Al_{0.65}Ga_{0.35}As films of a 500 Å-thickness 22b, and forms heterojunctions. In FIG. 4 the heterojunctions are partially shown. A P⁻GaAs contact layer 23 is formed in a thickness of 3000 Å on the photoabsorbing layer 22. An Al Schottky electrode 24 is mesh-patterned on the surface of the P⁻GaAs contact layer 23. On the surface of this P⁻GaAs contact layer 23 there is formed a very thin CsxOy film 25 by activating with Cs and O₂ for the reduction of a work function of the photemitting surface. An ohmic electrode 26 is formed on the underside of the P-GaAs substrate 21. A constant bias voltage is supplied by a power source 27 between the Schottky electrode 24 and the ohmic electrode 26.

FIG. 5 shows the band structure of the photoelectron emitting structure according to this embodiment with no bias voltage applied to. The respective layers in FIG. 5 has the same reference numerals as their corresponding layers in FIG. 4.

In this band structure, an energy difference between the conduction band of film 22a and the conduction band of film 22b is smaller than a minimum energy gap of the used semiconductors (undoped GaAs and Al_{0.65}Ga_{0.35}As) of the films 22a, 22b. Since each GaAs film 22a, which is a first semiconductor film, has a thickness of below 300 Å an electron state of which is quantized, the film 22a sandwiched by adjacent ones of the films 22b of Al_{0.65}Ga_{0.35}As, which is a second semiconductor film, functions as a potential well. Sub-bands are formed in each GaAs film 22a corresponding to a quantum level. At this time, since each Al_{0.65}Ga_{0.35}As layer 22b has a thickness above 45 Å which does not allow electrons to pass therethrough owing to the tunnel effect, the sub-bands in the film 22a are always filled with bound electrons.

The photoelectron emitting structure according to this embodiment is intended to further excite the bound electrons to sub-bands of other quantum levels by the absorption of the incident photons. It is evident that the photoelectron emitting structure according to this embodiment is intrinsically different from the conventional photoelectron emitting structure consisted of homogeneous semiconductive materials, the first conventional photoelectron emitting structure disclosed in Japanese Patent Laid-Open Publication No. 133633/1987, and the second conventional photoelectron emitting structure disclosed in Japanese Patent Laid-Open Publication No. 133634/1987, in which the absorption of the incident photons and the generation of photoelectrons are performed between the valence band and the conduction band. Accordingly the conventional photoelectron emitting structures are totally insensitive to the incident photons of wavelengths longer than λ=1.24/E_{g} which corresponds to an energy gap of the used semiconductors. But the photoelectron emitting structure according to this embodiment is sensitive to even to the incident photons of longer wavelengths than an energy gap of the used semiconductors. The wavelengths can be optionally varied by suitably designing the heterojunction of the semiconductor multi-layer of the photoabsorbing layer 22.

FIG. 6 shows the band structure of the photoelectron emitting structure according to this embodiment with a bias voltage applied to. In FIG. 6 as well the respective layers corresponding to the layers in FIG. 4 have the same reference numerals.

The photoelectrons generated between the sub-bands of the conduction bands of the GaAS films 22a of the photoabsorbing layer 22 by incident photons hν transfer to X valleys which are the bottoms of the conduction bands of the Al_{0.65}Ga_{0.35}As film 22b, which are a most lowest energy level. But since a 4 V-bias voltage is applied between the electrodes spaced from each other by 2.5 »m, and an electric field as high as about 1.6 KV/cm is formed, the generated photoelectrons are accelerated to immediately transit to Γ valleys which are higher energy bands. In this embodiment, where the Al_{0.65}Ga_{0.35}As film 22 b is an indirect transition semiconductor, such X-Γ transition takes place. Needless to say, when a direct transition semiconductor is used, the Γ-X transition or Γ-L transition takes place. These photoelectrons which have been thus accelerated by an internal electric field and transit to higher energy bands can arrive at the photoemitting surface without dropping into the potential wells of the GaAs films 22a because potential energies of the photoelectrons are retained sufficiently high when photoelectrons traverse the heterojunctions. A very small number of the photoelectrons which have arrived at the photoemitting surface are attracted to the Schottky electrode 24, but most of those photoelectrons pass through the electrode pattern and through a CsₓO_{y} film 25 to be emitted into a vacuum. At this time as potential energies of the photoelectrons are retained sufficiently high, the photoelectrons are efficiently emitted into a vacuum especially.

It is possible that the voltage to be applied between the electrodes is about 8 V to make an electric field as intense as about 3.2 KV/cm. The formation of an internal electric field in a range of 1 KV ∼ 55 KV/cm can cause the photoelectrons as mentioned above to be efficiently emitted into a vacuum. As described above, in the photoelectron emitting structure according to this embodiment, the photoelectrons generated by the incident photons between the sub-bands of the conduction band are accelerated by an internal electric field to transit the generated photoelectrons to higher energy bands and emit into a vacuum. That is, the photoelectron emitting structure according to this invention has an intrinsically different mechanism from, e.g., the photodetecting device reported by B. F. Levine et al. which uses the above-described third conventional quantum well, and in which photoelectrons are not accelerated by an internal electric field. In other words, in the photoelectron emitting structure according to this invention, an excitation of the incident photoelectrons takes place not between the so-called inter-bands of the valence band and the conduction band as conventionally, but between the sub-bands of the conduction band. Accordingly the photoelectron emitting structure according to this invention can be sensitive to long-wavelength light without the use of semiconductors of narrow energy gaps. Furthermore, the generated photoelectrons are accelerated by an internal electric field, and the photoelectrons which have fallen into the X valleys transit to the Γ valleys which have higher energy levels, after that the photoelectrons are emitted into a vacuum. As a result, as described above, the potential energy of the photoelectrons is higher than that of the conventional photoelectron emitting structures, and the generated photoelectrons can be excited to be efficiently emitted into a vacuum. Thus, the photoelectron emitting structure according to this invention has a very high sensitivity in comparison with that of the photoelectron emitting structures using the conventional structure of semiconductors. The photoelectron emitting structure according to this invention can set its wavelength limit at a very long wavelength. Furthermore, suitable designs of the kinds and structure of the heterojunction semiconductor multi-layer of the heterojunctions providing the photoabsorbing layer 22 can provide a photoelectron emitting structure which has a photodetecting characteristic having a peak at an optional wavelength. The photoelectron emitting structure according to this invention has high degrees of freedom of making choices of the semiconductor multi-layer in kinds, thicknesses and numbers of the semiconductor films, and accordingly can have the sensitivity adjusted to an optional one from a wide to a narrow range.

The secondary electron multiplication of the photoelectrons emitted into a vacuum makes it possible to provide long-wavelength photodetecting devices of high sensitivities and low noises which are operative at relatively high temperatures. That is, the photoelectron emitting structure according to the above-described embodiment is effectively applicable to electron tubes. In the application of a photocathode in photomultipliers, the photoelectron emitting structure according to the above-described embodiment is used as the photoelectric transfer surfaces, i.e., a photoemitting surface. The photoelectrons emitted from the photoemitting surface are secondary electron multiplied by the dynodes, and groups of the multiplied secondary electrons are detected by the anodes. In its application to image tubes the photoelectron emitting structure according to the above-described embodiment is used as a photoemitting surface in the image inputting units. The photoelectrons emitted from the photoemitting surface are focused by the electron lenses, and an image is formed on the phosphorous surface. The photoelectron emitting structure according to the above-described embodiment is applicable also to image intensifiers (I·I tubes) in which photoelectrons converged by the electron lenses are multiplied by the microchannel plates (MCPs). In its application to photo tubes, the photoelectron emitting structure according to the above-described embodiment is used as a photodetecting surface. The photoelectrons emitted from the photodetecting surface are detected by the anodes.

FIGs. 7, 8 and 9 show electron tubes each using the photoelectron emitting structure according to this invention. FIG. 7 is a sectional view of a side-on photomultiplier using a reflection-type photoemitting surface. FIG. 8 is a sectional view of a head-on photomultiplier using a transmission-type photoemitting surface. FIG. 9 is a sectional view of an image intensifier using a transmission-type photoemitting surface.

The photomultiplier of FIG. 7 includes in a vacuum vessel 71 a photoemitting surface 72, a plurality of dynodes 73, and an anode 74. On the front of the photoemitting surface 72 there is provided a mesh electrode 75. In the photomultiplier of FIG. 8, there is mounted a photoemitting surface 72 on one end of a vacuum vessel 71, and a focusing electrode 76 is provided in the vacuum vessel 71. In these respective photomultipliers photoelectrons (e⁻) are emitted by incident photons hν, and the photoelectrons are multiplied by the dynodes 73 and detected by the anode 74.

In the image intensifier of FIG. 9, a photoemitting surface 72 is secured to the opened front of a cylindrical bulb 81, and an glass output face plate 82 with a phosphorous film 83 applied to the inside thereof is secured to the opened rear end of the cylindrical bulb 81. Inside the cylindrical bulb 81 there is provided a microchannel plate 84.

These respective electron tubes using the photoelectron emitting structure according to this invention has a very high sensitivity especially in a long-wavelength range in comparison with the conventional electron tubes. Accordingly such electron tubes are very effective in the photometry, imaging, etc. at low illuminance.

In the above-described embodiment, the photoabsorbing layer 22 as the semiconductor multi-layer is formed of the heterojunction of the GaAs film 22a and Al0.65Ga0.35As film 22b but is not essentially limited to the heterojunction of these semiconductors. Other III-V compound semiconductors, or Si, Ge and their mixed crystal may be used. The kinds of the semiconductors are not essentially limited to two.

For example, the photoabsorbing layer 22 may be formed of GaAs films and AlAs films, or their mixed crystal. InP films and InGaAs films, or their mixed crystal may be used. InP films and AlGaAs films, or their mixed crystal may be used.

The formation of the photoabsorbing layer 22 of these materials can produce the same effects as in the above-described embodiment. Furthermore, the photoabsorbing layer may be formed of semiconductor multi-layer of the same kind having a p-n-i junction. In such case the same effects as those produced by the above-described embodiment can be achieved.

In the above-described embodiment, the Schottky electrode 24 is formed of Al, but the kind of the material of the Schottky electrode 24 is not specifically limited as long as the material is a metal which can form a good Schottky junction with used semiconductors. Its pattern can be optional.

The Schottky electrode 24 may be formed of, e.g., Ag, Au, Pt, Ti, W, Cr, WSi or alloys of these metals. The Schottky electrode of these metals can produce the same effects as those produced by the above-described embodiment.

In the above-described embodiment, the CsₓO_{y} film 25 is applied to the photoemitting surface of the photoelectron emitting structure for the reduction of the work function but the CsₓO_{y} film 25 is not essential. The film 25 may be formed of an alkali metal such as K, Na, Rb, Bi, Cs or others, or a compound, an oxide or a fluoride of any one of these metals.

These materials also can reduce the work function of the photoemitting surface.

## Claims

1. A photoelectron emitting structure for emitting therefrom photoelectrons generated by incident photons on a photoabsorbing layer (22),
the photoabsorbing layer formed of a semiconductor multi-layer comprising a plurality of semiconductor films (22a, 22b) including a first semiconductor film (22a) and a second semiconductor film (22b), the first semiconductor film (22a) with a narrow energy gap being formed in a thickness of below 300 Å which allows an electron state to be quantized, the second semiconductor film (22b) with a wide energy gap being formed in a thickness of above 45 Å which does not allow electrons to pass the second semiconductor film owing to the tunnel effect,
the absorption of the incident photons and the generation of electron-hole pairs taking place between sub-bands of a conduction band or between a sub-band and the bottom of a conduction band, of said first semiconductor film with the narrow energy gap,
wherein generated photoelectrons are accelerated by an internal electric field to transit to a higher energy band.

2. A photoelectron emitting structure according to claim 1, wherein the photoelectrons which have been excited to a lowest energy level of the conduction band are energized to transit to a higher energy level, and are accelerated by the internal electric field.

3. A photoelectron emitting structure according to claim 1, wherein an energy difference between lowest energy levels of the conduction bands formed in the respective semiconductor films making up the semiconductor multi-layer is smaller than the narrowest energy gap of the respective semiconductor films themselves.

4. A photoelectron emitting structure according to claim 1, wherein the first semiconductor film and the second semiconductor film are formed of different materials from each other and constitute a heterojunction.

5. A photoelectron emitting structure according to claim 4, wherein the semiconductor film layer are formed of III-V compound semiconductors, or their mixed crystal.

6. A photoelectron emitting structure according to claim 5, wherein the III-V compound semiconductors are GaAs and AlAs.

7. A photoelectron emitting structure according to claim 5, wherein the III-V compound semiconductors are InP and InGaAs.

8. A photoelectron emitting structure according to claim 5, wherein the III-V compound semiconductors are InP and AlGaAs.

9. A photoelectron emitting structure according to claim 1, wherein the first semiconductor film and the second semiconductor films are formed of semiconductors of the same kind doped with different conduction impurities, and form a homojunction.

10. A photoelectron emitting structure according to claim 9, wherein the semiconductor films are formed of Si, Ge, or its mixed crystal.

11. A photoelectron emitting structure according to claim 1, wherein on a surface thereof there are formed an electrode (24) for applying a required electric field to the photoabsorbing layer, and a metal film (25) for reducing a work function of the photoemitting surface.

12. A photoelectron emitting structure according to claim 11, wherein the electrode is in Schottky contact with the photoemitting surface.

13. A photoelectron emitting structure according to claim 12, wherein the electrode is formed of Al, Ag, Au, Pt, Ti, W, Cr or WSi, or a metal alloy of any one of these materials.

14. A photoelectron emitting structure according to claim 11, wherein the metal film is formed of K, Na, Rb, Bi or Cs, or a metal compound, an oxide or fluoride of any one of these materials.

15. An electron tube comprising a photoelectron emitting structure according to any one of claims 1 to 3.

16. A photodetector comprising an electron tube according to claim 15.

17. A photoelectron emitting device for emitting electrons in accordance with incident photons, comprising:
a semiconductor substrate (21);
a semiconductor multi-layer comprising a plurality of semiconductor films including a first semiconductor film (22a) and a second semiconductor film (22b), the first semiconductor film with a narrow energy gap having a thickness of below 300 Å, and the second semiconductor film with a wider energy gap having a thickness of above 45 Å;
a front surface electrode (24) formed on the semiconductor multi-layer;
a photoemitting unit including a backside electrode (26) formed on the backside of the semiconductor substrate; and
internal electric field generating means (27) for applying a voltage between the front surface electrode the backside electrode to generate an internal electric field in the semiconductor multi-layer.

18. A method for using a photoemitting device comprising:
a semiconductor substrate (21);
a semiconductor multi-layer comprising a plurality of semiconductor films influding a first semiconductor film (22a) and a second semiconductor film (22b), the first semiconductor film with a narrow energy gap having a thickness of below 300 Å, and the second semiconductor film with a wider energy gap having a thickness of above 45 Å;
a front surface electrode (24) formed on the semiconductor multi-layer;
a photoemitting unit including a backside electrode (26) formed on the backside of the semiconductor substrate; and
internal electric field generating means (27) for applying a voltage between the front surface electrode the backside electrode to generate an internal electric field in the semiconductor multi-layer, the method comprising:
applying a voltage between the front surface electrode and the backside electrode to generate an internal electric field in the semiconductor multi-layer, absorbing incident photons and generating electron-hole pairs between sub-bands of a conduction band of the energy band or between a sub-band and a bottom of the conduction band, of said first semiconductor film with a narrow energy gap, accelerating the generated photoelectrons by the internal electric field generated by the applied voltage to cause the photoelectrons to transit a higher energy band to be emitted.

19. A photoelectron emitting structure comprising a photon-absorbing layer (22) comprising a stack of semiconductor layers, each semiconductor layer comprising a first semiconductor film (22a) having a relatively narrow energy gap and a thickness of less than 300Å and a second semiconductor film (22b) having a relatively wide energy gap and a thickness of more than 45Å, the structure further comprising electrodes (24,26) sandwiching the photon-absorbing layer (22) between which electrodes a voltage can be applied for the generation of an internal electric field.

## Patentansprüche

1. Photoelektronen emittierende Struktur zum Emittieren von durch auf eine photoabsorbierende Schicht (22) einfallende Photonen erzeugten Photoelektronen von der Struktur,
wobei die aus einem Halbleiter-Vielschichtsystem gebildete photoabsorbierende Schicht eine Vielzahl von Halbleiterfilmen (22a, 22b) mit einem ersten Halbleiterfilm (22a) und einem zweiten Halbleiterfilm (22b) umfaßt und der erste Halbleiterfilm (22a) mit einer engen Energielücke in einer Dicke von unterhalb 300 Å gebildet ist, was zuläßt, daß ein Elektronenzustand quantisiert ist, der zweite Halbleiterfilm (22b) mit einer breiten Energielücke in einer Dicke von oberhalb 45 Å gebildet ist, was nicht zuläßt, daß Elektronen aufgrund des Tunneleffekts durch den zweiten Halbleiterfilm durchgehen,
wobei die Absorption der einfallenden Photonen und die Erzeugung von Elektron-Loch-Paaren zwischen Subbändern eines Leitungsbands oder zwischen einem Subband und dem Boden eines Leitungsbands des ersten Halbleiterfilms mit der engen Energielücke stattfindet,
worin erzeugte Photoelektronen durch ein inneres elektrisches Feld beschleunigt werden, wobei sie zu einem höheren Energieband übergehen.

2. Photoelektronen emittierende Struktur nach Anspruch 1, bei der die Photoelektronen, die zu einem untersten Energieniveau des Leitungsbandes angeregt worden sind, angeregt werden, so daß sie zu einem höheren Energieniveau übergehen und durch das innere elektrische Feld beschleunigt werden.

3. Photoelektronen emittierende Struktur nach Anspruch 1, bei der eine Energiedifferenz zwischen den untersten Energieniveaus der Leitungsbänder, die in den jeweiligen Halbleiterfilmen, die das Halbleiter-Vielschichtsystem aufbauen, gebildet sind, kleiner als die engste Energielücke der jeweiligen Halbleiterfilme selbst ist.

4. Photoelektronen emittierende Struktur nach Anspruch 1, bei der der erste Halbleiterfilm und der zweite Halbleiterfilm aus voneinander unterschiedlichen Materialien gebildet sind und einen Heteroübergang darstellen.

5. Photoelektronen emittierende Struktur nach Anspruch 4, bei der die Halbleiterfilmschicht aus III-V-Verbindungshalbleitern oder ihren Mischkristallen gebildet ist.

6. Photoelektronen emittierende Struktur nach Anspruch 5, bei der die III-V-Verbindungshalbleiter GaAs und AlAs sind.

7. Photoelektronen emittierende Struktur nach Anspruch 5, bei der die III-V-Verbindungshalbleiter InP und InGaAs sind.

8. Photoelektronen emittierende Struktur nach Anspruch 5, bei der die III-V-Verbindungshalbleiter InP und AlGaAs sind.

9. Photoelektronen emittierende Struktur nach Anspruch 1, bei der der erste Halbleiterfilm und der zweite Halbleiterfilm aus Halbleitern von derselben Art gebildet sind, die mit unterschiedlichen Leitfähigkeits-Verunreinigungen dotiert sind, und einen Homoübergang bilden.

10. Photoelektronen emittierende Struktur nach Anspruch 9, bei der die Halbleiterfilme aus Si, Ge oder ihrem Mischkristall gebildet sind.

11. Photoelektronen emittierende Struktur nach Anspruch 1, bei der eine Elektrode (24) zum Anlegen eines erforderlichen elektrischen Feldes an die photoabsorbierende Schicht und ein Metallfilm (25) zum Verringern der Austrittsarbeit der photoemittierenden Oberfläche auf einer Oberfläche der Photoelektronen emittierenden Struktur gebildet sind.

12. Photoelektronen emittierende Struktur nach Anspruch 11, bei der die Elektrode in Schottky-Kontakt mit der photoemittierenden Oberfläche ist.

13. Photoelektronen emittierende Struktur nach Anspruch 12, bei der die Elektrode aus Al, Ag, Au, Pt, Ti, W, Cr oder WSi oder einer Metallegierung aus einem dieser Materialien gebildet ist.

14. Photoelektronen emittierende Struktur nach Anspruch 11, bei der der Metallfilm aus K, Na, Rb, Bi oder Cs oder einer Metallverbindung, einem Oxid oder Fluorid aus einem dieser Materialien gebildet ist.

15. Elektronenröhre mit einer Photoelektronen emittierenden Struktur nach einem der Ansprüche 1 bis 3.

16. Photodetektor mit einer Elektronenröhre nach Anspruch 15.

17. Photoelektronen emittierende Struktur zum Emittieren von Elektronen gemäß einfallenden Photonen, umfassend:
ein Halbleiter-Substrat (21);
ein Halbleiter-Vielschichtsystem mit einer Vielzahl von Halbleiterfilmen, umfassend einen ersten Halbleiterfilm (22a) und einen zweiten Halbleiterfilm (22b), wobei der erste Halbleiterfilm mit einer engen Energielücke eine Dicke von unterhalb 300 Å hat und der zweite Halbleiterfilm mit einer breiteren Energielücke eine Dicke von oberhalb 45 Å hat;
eine vordere Oberflächenelektrode (24), die auf dem Halbleiter-Vielschichtsystem gebildet ist;
eine photoemittierende Einheit mit einer rückseitigen Elektrode (26), die auf der Rückseite des Halbleitersubstrats gebildet ist; und
Einrichtungen (27) zur Erzeugung eines inneren elektrischen Feldes zum Anlegen einer Spannung zwischen der vorderen Oberflächenelektrode und der rückseitigen Elektrode, wobei ein inneres elektrisches Feld in dem Halbleiter-Vielschichtsystem erzeugt wird.

18. Verfahren zur Verwendung einer photoemittierenden Vorrichtung, umfassend:
ein Halbleiter-Substrat (21);
ein Halbleiter-Vielschichtsystem mit einer Vielzahl von Halbleiterfilmen, umfassend einen ersten Halbleiterfilm (22a) und einen zweiten Halbleiterfilm (22b), wobei der erste Halbleiterfilm mit einer engen Energielücke eine Dicke von unterhalb 300 Å hat und der zweite Halbleiterfilm mit einer breiteren Energielücke eine Dicke von oberhalb 45 Å hat;
eine vordere Oberflächenelektrode (24), die auf dem Halbleiter-Vielschichtsystem gebildet ist;
eine photoemittierende Einheit mit einer rückseitigen Elektrode (26), die auf der Rückseite des Halbleitersubstrats gebildet ist; und
Einrichtungen (27) zur Erzeugung eines inneren elektrischen Feldes zum Anlegen einer Spannung zwischen der vorderen Oberflächenelektrode und der rückseitigen Elektrode, wobei ein inneres elektrisches Feld in dem Halbleiter-Vielschichtsystem erzeugt wird,
wobei das Verfahren die folgenden Schritte umfaßt:
Anlegen einer Spannung zwischen der vorderen Oberflächenelektrode und der rückseitigen Elektrode, um ein inneres elektrisches Feld in dem Halbleiter-Vielschichtsystem zu erzeugen, Absorbieren einfallender Photonen und Erzeugen von Elektron-Loch-Paaren zwischen Subbändern eines Leitungsbands des Energiebands oder zwischen einem Subband und einem Boden des Leitungsbands des ersten Halbleiterfilms mit einer engen Energielücke, Beschleunigen der erzeugten Photoelektronen durch das innere elektrische Feld, das durch die angelegte Spannung erzeugt wird, wobei bewirkt wird, daß die Photoelektronen zu einem höheren Energieband übergehen, wobei sie emittiert werden.

19. Photoelektronen emittierende Struktur mit einer Photonen absorbierenden Schicht (22), umfassend eine Aufschichtung aus Halbleiterschichten, wobei jede Halbleiterschicht einen ersten Halbleiterfilm (22a) mit einer relativ engen Energielücke und einer Dicke von weniger als 300 Å und einen zweiten Halbleiterfilm (22b) mit einer relativ breiten Energielücke und einer Dicke von mehr als 45 Å umfaßt, wobei die Struktur ferner Elektroden (24, 26) für die Erzeugung eines inneren elektrischen Feldes umfaßt, die die Photonen absorbierende Schicht (22) sandwichartig umgeben und wobei zwischen diesen Elektroden eine Spannung angelegt werden kann.

## Revendications

1. Structure d'émission de photoélectrons pour l'émission de photoélectrons générés par des photons incidents sur une couche photo-absorbante (22), la couche photo-absorbante formée d'une multicouche à semi-conducteur comprenant une pluralité de films de semi-conducteur (22a, 22b) comprenant un premier film de semi-conducteur (22a) et un second film de semi-conducteur (22b), le premier film de semi-conducteur (22a) possédant un intervalle d'énergie étroit formé dans une épaisseur inférieure à 300 Å, ce qui permet la quantification d'un état électronique, le second film de semi-conducteur (22b) possédant un large intervalle d'énergie formé dans une épaisseur en dessous de 45 Å, ce qui permet aux électrons de passer le second film de semi-conducteur par l'effet de tunnel, l'absorption des photons incidents et la génération de paires d'électron/trou ayant lieu entre les sous-bandes d'une bande de conduction ou entre une sous-bande et le bas d'une bande de conduction dudit premier film de semi-conducteur à intervalle d'énergie étroit,
structure dans laquelle les photoélectrons sont accélérés par un champ électrique interne pour passer sur une plus haute bande d'énergie.

2. Structure d'émission de photoélectrons selon la revendication 1, dans laquelle les photoélectrons qui sont excités à un plus bas niveau d'énergie de la bande de conduction sont activés pour transiter sur un plus haut niveau d'énergie, et sont accélérés par le champ électrique interne.

3. Structure d'émission de photoélectrons selon la revendication 1, dans laquelle une différence d'énergie entre les plus bas niveau d'énergie des bandes de conduction formées dans les films respectifs de semi-conducteur constituant la multicouche de semi-conducteur est plus faible que l'intervalle d'énergie le plus étroit des films respectifs de semi-conducteur eux-mêmes.

4. Structure d'émission de photoélectrons selon la revendication 1, dans laquelle le premier film de semi-conducteur et le second film de semi-conducteur sont formés de matériaux différents l'un de l'autre et constituent une hétéro-jonction.

5. Structure d'émission de photoélectrons selon la revendication 4, dans laquelle les couches de film de semi-conducteur sont formées de semi-conducteurs de composé III-V ou de leur mélange cristallin.

6. Structure d'émission de photoélectrons selon la revendication 5, dans laquelle les semi-conducteurs de composé III-V sont le GaAs et l'AlAs.

7. Structure d'émission de photoélectrons selon la revendication 5, dans laquelle les semi-conducteurs de composé III-V sont l'InP et l'InGaAs.

8. Structure d'émission de photoélectrons selon la revendication 5, dans laquelle les semi-conducteurs de composé III-V sont l'InP et l'AlGaAs.

9. Structure d'émission de photoélectrons selon la revendication 1, dans laquelle le premier film de semi-conducteur et le second film de semi-conducteur sont formés de semi-conducteurs du même type de dopage avec différentes impuretés de conduction et forment une homo-jonction.

10. Structure d'émission de photoélectrons selon la revendication 9, dans laquelle les films de semi-conducteur sont formés de Si, de Ge ou de leur mélange cristallin.

11. Structure d'émission de photoélectrons selon la revendication 1, dans laquelle sont formés, en surface, une électrode (24) pour l'application d'un champ électrique requis à la couche photo-absorbante et un film de métal (25) pour réduire une fonction de charge de la surface photoémettrice.

12. Structure d'émission de photoélectrons selon la revendication 11, dans laquelle l'électrode est en contact de Schottky avec la surface photoémettrice.

13. Structure d'émission de photoélectrons selon la revendication 12, dans laquelle l'électrode est formée de Al, Ag, Au, Pt, Ti, W, Cr ou de WSi ou d'un alliage métallique de l'un quelconque de ces matériaux.

14. Structure d'émission de photoélectrons selon la revendication 11, dans laquelle le film de métal est formé de K, Na, Rb, Bi ou de Cs ou d'un composé de métal, d'un oxyde ou d'un fluorure de l'un quelconque de ces matériaux.

15. Tube électronique comprenant une structure d'émission de photoélectrons selon l'une quelconque des revendications 1 à 3.

16. Photodétecteur comprenant un tube electronique selon la revendication 15.

17. Dispositif d'émission de photoélectrons pour émettre des électrons selon des photons incidents, comprenant :
- un support de semi-conducteur (21);
- une multicouche de semi-conducteur comprenant une pluralité de films de semi-conducteur comprenant un premier film de semi-conducteur (22a) et un second film de semi-conducteur (22b), le premier film de semi-conducteur présentant un intervalle d'énergie étroit ayant une épaisseur inférieure à 300 Å, et le second film de semi-conducteur ayant un plus large intervalle d'énergie présentant une épaisseur supérieure à 45 Å;
- une électrode de surface avant (24) formée sur la multicouche de semi-conducteur;
- une unité photoémettrice comprenant une électrode arrière (26) formée sur le côté arrière du support de semi-conducteur; et
- un moyen de génération de champ électrique interne (27) pour l'application d'une tension entre l'électrode de surface avant et l'électrode de côté arrière afin de générer un champ électrique interne dans la multicouche de semi-conducteur.

18. Procédé pour l'utilisation d'un dispositif photoémetteur comprenant :
- un support de semi-conducteur (21);
- une multicouche de semi-conducteur comprenant une pluralité de films de semi-conducteur comprenant un premier film de semi-conducteur (22a) et un second film de semi-conducteur (22b), le premier film de semi-conducteur présentant un intervalle d'énergie étroit ayant une épaisseur inférieure à 300 Å, et le second film de semi-conducteur ayant un plus large intervalle d'énergie présentant une épaisseur supérieure à 45 Å;
- une électrode de surface avant (24) formée sur la multicouche de semi-conducteur;
- une unité photoémettrice comprenant une électrode arrière (26) formée sur le côté arrière du support de semi-conducteur; et
- un moyen de génération de champ électrique interne (27) pour l'application d'une tension entre l'électrode de surface avant et l'électrode de côté arrière afin de générer un champ électrique interne dans la multicouche de semi-conducteur,
procédé comprenant l'application d'une tension entre l'électrode de surface avant et l'électrode de côté arrière pour générer un champ électrique interne dans la multicouche de semi-conducteur, l'absorption des photons incidents et la génération de paires d'électron/trou entre des sous-bandes d'une bande de conduction de la bande d'énergie ou entre une sous-bande et le bas de la bande de conduction dudit premier film de semi-conducteur ayant un intervalle d'énergie étroit, l'accélération des photoélectrons générés par le champ électrique interne lui-même généré par la tension appliquée pour provoquer la transition des photoélectrons à émettre sur une plus haute bande d'énergie.

19. Structure d'émission de photoélectrons comprenant une couche photo-absorbante (22) comprenant une pile de couches de semi-conducteur, chaque couche de semi-conducteur comprenant un premier film de semi-conducteur (22a), possédant un intervalle d'énergie relativement étroit et une épaisseur inférieure à 300 Å, et un second film de semi-conducteur (22b), possédant un intervalle d'énergie relativement grand et une épaisseur dépassant 45 Å, structure comprenant, de plus, des électrodes (24, 26) prenant en sandwich la couche photo-absorbante (22), électrodes entre lesquelles une tension peut être appliquée pour la génération d'un champ électrique interne.
